

Aug. 23, 1949.

J. E. FLOOD  
METHOD OF COVERING A WIRE HAVING  
INTERSTICES THEREIN  
Filed Nov. 27, 1945

2,479,919

Fig. 1



Fig. 2



Fig. 3



Fig. 4



Fig. 5



Fig. 6



INVENTOR  
James E. Flood  
BY *Johnson, Klein and French*

ATTORNEYS

## UNITED STATES PATENT OFFICE

2,479,919

METHOD OF COVERING A WIRE HAVING  
INTERSTICES THEREINJames E. Flood, Norwich, Conn., assignor to The  
Plastic Wire & Cable Corporation, Norwich,  
Conn., a corporation of Connecticut

Application November 27, 1945, Serial No. 631,116

5 Claims. (Cl. 18—59)

1

The present invention relates to method of making a covered wire and particularly to the securing of an extruded covering of thermoplastic resinous synthetic polymers such as polyvinyl chloride, copolymers of polyvinyl chloride such as copolymers of vinyl chloride-vinyl acetate, polyethylene, nylon and the like, to the wire.

I have found that in extruding such covering material about a wire that the cover, while closely embracing the wire, retains its tubular form and does not satisfactorily bond or adhere to the wire as do vulcanizable compounds such as rubber or the like and that it slides on the wire when the wire is anchored and a pull is given to the covering. This has been true even when the wire is covered with a cotton wrap or when stranded wire has been used.

The present invention overcomes these difficulties by providing a mechanical interlock between the cover and the wire which is substantial and will hold the insulation against longitudinal displacement on the wire.

The mechanical interlock has been accomplished by rendering fluid a quantity of the cover material and applying a relatively thin coating thereof to the wire so that it penetrates the interstices of the wire or covering thereabout. When this coating hardens, it will be mechanically interlocked with the wire or wrapping and be secured thereto. The required quantity of cover material is then extruded over the thin coating on the wire and the two become integrally united into a single cover which is mechanically interlocked with the wire.

The cover material may be rendered fluid in many ways. In one form of the invention the cover material is mixed with a solvent therefor which is driven off after the material is applied to the wire leaving the solid interlocked coating on the wire.

According to another form of the invention, the unplasticized cover material is dispersed in a compatible liquid plasticizer in a suitable mixture under controlled conditions. The material is one in which the mixing cycle is not quite complete so that it remains as a heavy liquid coating when applied to the wire.

According to the present invention the coating mechanically connected to the wire completely loses its identity as a coating when the jacket of

2

hot cover material is applied thereto and merges with and forms an integral part thereof.

The present invention is of particular advantage in connection with securing extruded thermoplastic resinous synthetic polymers as insulation on electrical conductors to provide the necessary interlock to enable the cords made therefrom to withstand the pulls thereon in use.

While it is preferred to use the cover material in making the coating composition, it is to be understood that other compatible materials may be used.

Other advantages will be apparent from the specification and claims when considered with the drawings in which:

Figure 1 is a side elevation of a wire having a coating thereon.

Fig. 2 is a section taken along line 2—2 of Fig. 1.

Fig. 3 is a side elevation of a wire having a cover thereon.

Fig. 4 is a section taken along line 4—4 of Fig. 3.

Fig. 5 is a view showing a wrapped wire.

Fig. 6 is a section taken along line 6—6 of Fig. 5.

The present invention will be described in connection with the application of a covering of insulation to an electrical conductor. However, it is to be understood that wires other than conductors may be covered for various other purposes.

As shown in the drawings, a wire 10 has a covering 11 extruded thereover. When the cover material comprises a synthetic resinous polymer, such as polyvinyl chloride or copolymers thereof such as copolymers of vinyl chloride-vinyl acetate, polyethylene, nylon and the like which are water repellent and have good insulating properties, it has been found that these materials will not bond with the wire but form a spaghetti-like mass around the wire which will readily slip with respect to the wire. This is particularly true when the conductor is used in a cord set and the wire anchored to the attaching connector or plug. Under these circumstances, when the wire is gripped and pulled to remove the connector, as is usually the case, the insulation slides relative to the wire and produces a bare portion which renders such cords unfit for use.

In order to securely anchor the insulation to the wire according to the present invention a wire having interstices therein is employed. At

present preferred this may be a twisted or braided stranded wire or a smooth wire 10a having a wrap or braid of cotton 13 thereon which will provide interstices through which a mechanical interlock between the insulation and the wire may be achieved. The term "wire" shall be used to designate both stranded or wrapped wire, singly or in multiples thereof.

The interlock, according to the present invention, is accomplished by preparing a coating of the insulation material which is sufficiently fluid that it will penetrate the interstices of the wire and become mechanically interlocked and anchored thereto.

The coating may be formed by mixing some of the insulation material with a suitable solvent, for example when vinyl chloride or the copolymer of vinyl chloride-vinyl acetate are used, acetone, methyl ethyl ketone, cyclohexanone or mixtures thereof may be mixed therewith to render the same liquid. The viscosity of the liquid may be adjusted as required for the particular need. The wire 10 is run through a bath of the coating material which penetrates the interstices and applies a thin coating over the wire. The solvent is then allowed to evaporate or is driven off by means of heat or the like, leaving behind a very thin coating 12 of the compound mechanically anchored to the conductor or wrap thereabout as shown in Figs. 1 and 2.

The coated wire may pass through an oven or other heating means and the outer surfaces softened before it is fed to the cover or jacket extruding machine. However, I have found that with most compositions, when the coated wire is passed through the extruding machine and the cover or jacket of hot insulating material extruded directly on the coating, the heat of the cover material will be sufficient to melt the surface of the coating and cause it to become integral with the extruded insulation. As shown in Fig. 4 the coating and jacket of insulation form a unified cover of insulation which is anchored to the interstices in the wire and which will hold the insulation against slipping on the wire.

It is preferable that the coating be thermoplastic at a somewhat lower temperature than the cover material so that it will readily melt and blend in with the jacket of cover material as it is extruded thereover. The heat of the jacket while sufficient to plasticize or soften the outer portion of the coating does not affect the portion of the coating which extends into the interstices and locks the coating to the wire so that when the insulating cover hardens it is securely mechanically connected to the wire.

Polyethylene and a suitable solvent therefor may be employed in a similar manner to provide a coating and the extruded cover.

The coating may also be formed by a quantity of the unplasticized resin such as polyvinyl chloride or copolymer of vinyl chloride-vinyl acetate, which is dispersed in a compatible liquid plasticizer in a suitable mixer and under controlled conditions. Such plasticizers may be dibutyl phthalate, diethyl phthalate or others. The resin is ground in the plasticizer until a smooth uniform constant dispersion is formed. The mixture is a heavy liquid composition in which the mixing cycle is not complete, i. e. there is not a complete fluxing of the plasticizer and the resin.

The wire is run through a bath of the coating composition and the material is applied to the wire and penetrates into the interstices. The excess is wiped off. The bath is located behind the

extruder so that the wire then passes into the extruder where the hot jacket of insulation or cover material is extruded thereover. The heat of the jacket causes the coating to change phase, i. e., to complete the fluxing and change from a heavy liquid to an elastic solid and the jacket being of a similar composition and in a hot plastic state becomes fused with the coating into a solid mass which has portions interlocked with the conductor.

The coating materials and the cover may, of course, have suitable oils, pigments, stabilizers included in the mixture as required by the particular purpose for which the wire is to be used.

While I prefer to use the same material in the coating as in the cover, it is to be understood that other compatible materials which will fuse together to form an integral cover may be used.

Variations and modifications may be made within the scope of this invention and portions of the improvements may be used without others.

I claim:

1. A method of covering a wire comprising coating a wire having interstices therein with an unheated fluid coating composition of thermoplastic resinous synthetic polymer to cause the composition to enter said interstices and interlock therewith, and extruding a plastic jacket of cover material of the same thermoplastic resinous synthetic polymer in hot plastic form over the coating, the cover material and coating becoming an integral cover mechanically secured to the wire.

2. A method of covering a wire comprising coating a wire having interstices therein with an unheated fluid coating of cover composition to cause the composition to enter said interstices and interlock therewith, and extruding a jacket of the same cover material in hot plastic form over the coating, the hot cover material causing the coating to become fused therewith into an integral cover.

3. A method of insulating a conductor comprising mixing a thermoplastic resinous synthetic polymer with a solvent to form a fluid coating composition, coating a wire having interstices therein with said composition to cause the composition to enter said interstices; driving off the solvent to leave a thin coat of coating material on the wire and interlock therewith; and extruding a jacket of cover material of the same polymer in hot plastic form over the coating, the hot cover material causing the surface of the coating to become soft and fuse therewith into an integral cover.

4. A method of insulating a conductor comprising mixing a thermoplastic resinous synthetic polymer cover material with a solvent to form a fluid coating composition, coating a wire having interstices therein with said composition to cause the composition to enter said interstices; driving off the solvent to leave a thin coat of coating material on the wire and interlock therewith; and softening the surface of the coating and extruding a jacket of cover material of the same polymer in hot plastic form over the coating, the hot cover material and the coating becoming fused into an integral cover.

5. A method of insulating a conductor comprising mixing a thermoplastic resinous synthetic polymer with a plasticizer to form a liquid coating composition having an incomplete fluxing of the plasticizer and said polymer, coating a wire having interstices therein with said composition to cause the composition to enter said inter-

stices; and extruding a jacket of cover material of a compatible polymer capable of uniting by fusion with said synthetic polymer in hot plastic form over the coating, the hot cover material causing the coating to complete the fluxing of the plasticizer and polymer and change phase from a heavy liquid to an elastic solid and fuse with the cover material into an integral cover.

JAMES E. FLOOD.

**REFERENCES CITED**

The following references are of record in the file of this patent:

UNITED STATES PATENTS

| Number    | Name                 | Date          |
|-----------|----------------------|---------------|
| 2,249,280 | Koch -----           | July 15, 1941 |
| 2,308,638 | Balthis et al. ----- | Jan. 19, 1943 |
| 2,312,024 | Brown -----          | Feb. 23, 1943 |
| 2,332,538 | Smith -----          | Oct. 26, 1943 |
| 2,384,224 | Williams -----       | Sept. 4, 1945 |

FOREIGN PATENTS

| Number     | Country             | Date         |
|------------|---------------------|--------------|
| 10 190,778 | Great Britain ----- | Dec. 2, 1922 |